



US006340658B1

(12) **United States Patent**  
Cannon et al.

(10) **Patent No.:** US 6,340,658 B1  
(45) **Date of Patent:** Jan. 22, 2002

(54) **VEGETABLE-BASED TRANSFORMER OIL AND TRANSMISSION LINE FLUID**

(75) Inventors: **Glenn S. Cannon**, Waverly, IA (US);  
**John A. Kotowski**, Piedmont, CA (US)

(73) Assignee: **Waverly Light and Power**, Waverly, IA (US)

(\*) Notice: Subject to any disclaimer, the term of this patent is extended or adjusted under 35 U.S.C. 154(b) by 0 days.

(21) Appl. No.: **09/705,015**

(22) Filed: **Nov. 2, 2000**

**Related U.S. Application Data**

(63) Continuation-in-part of application No. 09/335,990, filed on Jun. 18, 1999, now Pat. No. 6,159,913, which is a continuation of application No. 09/075,963, filed on May 11, 1998, now Pat. No. 5,958,851.

(51) **Int. Cl.**<sup>7</sup> ..... **C10M 105/32; H01B 3/20**

(52) **U.S. Cl.** ..... **508/491; 508/578; 252/570; 252/579; 174/17 LF; 361/327**

(58) **Field of Search** ..... 508/491

(56) **References Cited**

**U.S. PATENT DOCUMENTS**

1,776,309 A \* 9/1930 Clark ..... 252/407  
3,928,705 A \* 12/1975 Loft et al. ..... 252/567  
4,421,663 A \* 12/1983 Embree et al. ..... 252/74  
4,536,331 A \* 8/1985 Shedigian ..... 252/579  
4,543,207 A \* 9/1985 Sato et al. ..... 252/570  
4,642,730 A \* 2/1987 Sato et al. ..... 252/570  
4,734,824 A \* 3/1988 Sato et al. ..... 361/315

4,791,240 A \* 12/1988 Marin et al. ..... 252/570  
4,812,262 A \* 3/1989 Shinzawa et al. ..... 252/567  
4,931,900 A \* 6/1990 Lobo et al. ..... 252/579  
5,077,069 A \* 12/1991 Chang et al. ..... 426/330.6  
5,413,725 A \* 5/1995 Lal et al. ..... 508/491  
5,451,334 A \* 9/1995 Bongardt et al. ..... 508/307  
5,595,966 A \* 1/1997 Rees et al. ..... 508/591  
5,766,517 A \* 6/1998 Goedde et al. ..... 252/570  
5,958,851 A \* 9/1999 Cannon et al. ..... 508/491  
5,981,781 A \* 11/1999 Knowlton ..... 554/224  
6,037,537 A \* 3/2000 McShane et al. ..... 174/17 LF  
6,159,913 A \* 12/2000 Cannon et al. ..... 508/491  
6,274,067 B1 8/2001 Oommen et al.

\* cited by examiner

*Primary Examiner*—Ellen M. McAvoy

(74) *Attorney, Agent, or Firm*—Zarley, McKee, Thomte, Voorhees & Sease

(57)

**ABSTRACT**

A vegetable oil-based electrically-insulating fluid. This fluid is environmentally-friendly and has a high flash point and a high fire point. The base oil is hydrogenated to produce maximum possible stability of the oil, or alternatively, is a higher oleic acid oil. The vegetable oils of the preferred embodiments are soybean or corn oils. The oil can be winterized to remove crystallized fats and improve the pour point of the base oil, without the necessity of heating the oil. The base oil can also be combined with an additive package containing materials specifically designed for improved pour point, improved cooling properties, and improved dielectric stability. The fluid is useful in electrical components such as transformers and transmission lines. The invention also provides methods for making the fluid and fluid-filled electrical components.

**57 Claims, 1 Drawing Sheet**





Fig. 1



Fig. 2

- - Unused
- - After a 1000 hour pump test

## VEGETABLE-BASED TRANSFORMER OIL AND TRANSMISSION LINE FLUID

### CROSS-REFERENCE TO RELATED APPLICATION

This as a continuation-in-part of application Ser. No. 09/335,990, filed Jun. 18, 1999, now U.S. Pat. No. 6,159,913, which is a continuation of application Ser. No. 09/075,963, filed May 11, 1998, U.S. Patent No. 5,958,851.

### BACKGROUND OF THE INVENTION

#### 1. Field of the Invention

The present invention relates to fluids that are used with electrical equipment and transmission components, and in particular, to fluids used for electrical insulation and/or heat dissipation in electrical components, such as, for example, electrical transformers and electrical transmission lines.

#### 2. Problems in the Art

The components that are used to generate and transfer electrical energy to end users, such as homeowners or businesses, are well known in the art. Electrical power producers generally generate electrical power at very high initial voltages. Handling of such high voltages requires substantial electrical insulation. It requires control of heat that is generated from the transmission of the electrical energy and maintenance of its dielectric properties.

It has been found that certain fluids have high insulating and heat dissipation properties. These fluids are used with such electrical components as transformers and fluid-filled transmission lines. One particular problem is that over time and with substantial exposure to high-voltage electricity the beneficial characteristics of such fluids, such as insulating and/or heat dissipation properties, degrade.

Conventionally, petroleum-based fluids are used for these types of applications. It must be appreciated that such fluids have certain properties that allow them to function satisfactorily. They must be electrically-insulating and dissipate heat. They must resist break-down. Synthetic fluids are also in use. However, currently used fluids have several deficiencies or concerns.

Most of the current fluids are minimally biodegradable. They pose safety or contamination concerns as they can be toxic to humans and animals. Many electrical components holding such fluids are situated near water or waterways. Leakage or spills can cause serious damage to water and marine life. Leaks or spills on land can threaten groundwater and contaminate soil.

Petroleum-based products are non-renewable. The amount of fluid of this type in use is significant. For example, one 15 MVA transformer (approximately serves 2000 customers, both residential and commercial) requires on the order of 3600 gallons of electrically-insulating fluid. One mile of fluid-filled transmission cable (6 inch diameter) requires about 7000 gallons. About 4.5 billion gallons of transformer oil are currently in use in the U.S. There are approximately 20,000 miles of high-pressure fluid-filled transmission cables (one type of the same) in the United States, most in larger cities and, therefore, most are near water or waterways.

As can be appreciated, significant amounts of resources, both time and money, are spent by electrical power companies in designing and implementing plans and systems to deter leaks or spills and to monitor transformers and transmission cables of these types for leaks or spills. It is estimated such costs are in the millions of dollars in the

United States. Additionally, substantial resources are expended in reporting leaks or spills, even minor, because of environmental rules and regulations with regard to at least petroleum-based fluids. Of course, the effect of leaks or spills themselves can be very costly, as can remediation of the same.

Therefore, there have been attempts to look to new sources for such fluids, including vegetable oils. Such attempts would address both the environmental concerns as well as the issue of renewability of source as well as the potential for recycling into greases, for example, after use.

A similar problem exists with respect to petroleum- or synthetic-based lubricants. The idea of substituting vegetable oils for petroleum-based industrial lubricants is not new. Furthermore, finite supply of petroleum-based products, oil importation concerns, and concerns over environmental effects from spills/disposal of petroleum-based lubricants has fueled interest in the use of vegetable oils as viable substitutes.

Efforts to use vegetable oils as a substitute have focused upon less stringent uses such as hydraulic fluids, transmission fluids, and greases and not on the more severe automotive-type (engine) lubricants or transformer cooling oils. The vast majority of these endeavors have utilized vegetable oils high in natural oleic acid levels such as safflower oil, canola and rapeseed oils. The reason for the focused research upon these high oleic acid level vegetable oils is the tendency of natural vegetable oils to destabilize in use absent the presence of a high level of oleic acid. Other vegetable oils, such as soybean and corn oils, have a relatively low level of oleic acid and have been uniformly rejected in practical application because of the tendency of these oils to solidify while in use within the environment of high temperatures.

There are several fundamental properties transformer oils, for example, require, most of which are contrary to the natural properties of vegetable oils. These properties are oxidation stability, dielectric constant, pour point, sludge formation, and formation of acids. Of the vegetable oils, such as rapeseed, canola, and castor, commonly considered for industrial lubricants, soybean and corn oils are the more unstable (oxidatively) because of their unsaturated nature.

The primary purpose of the types of fluid needed for electrical transformers and fluid-filled transmission lines, hereinafter referred to as electrically-insulating fluid, is to maintain cooling properties and fluid characteristics while in use within the system so as to maintain appropriate temperature, as well as dielectric strength, on demand. The heat of the transformer unit, for example, can increase to high levels for extended periods of time which the fluid must be able to tolerate without losing its properties. Additionally, the operation of transformers and the process of heat dissipation at varied ambient temperatures subjects the fluid to constant stresses.

Some vegetable oil-based electrically-insulating fluids have found commercial success. These vegetable oil-based fluids have often been of the more naturally stable seed oils. Specifically, oils naturally high in oleic acid content or low in linolenic content, and in some cases low erucic acid, have been used. Variations in temperature, in particular high temperature environments, are known to impact the ability of a vegetable oil-based fluid to remain in the liquid state. As a result, this limited number of vegetable oils have been found to function with relative success.

Use of vegetable oil-based electrically-insulating fluids in the outdoors environment presents a much harsher chal-

lengue. To date, the success of such fluids has been very limited. Rapeseed and canola oil-based fluids have been commercially offered, but questions remain as to the functionality. These questions include sufficiency of electrical insulating properties and oxidation problems. Also, since crops such as rapeseed and canola are grown mainly outside the United States, it is expensive to import and produce which in turn increases the expense of making oils from them.

Because the above questions regarding rapeseed and canola oil exist, the same questions exist with respect to other less thermally stable oils, such as soybean and corn.

Soybean and corn oils, because of their unsaturated natures, lack desired oxidative stability for many industrial applications where continuous long-term heating takes place. In use, transformer and transmission line cooling oil must successfully operate not only to cool the components of the transformer and transmission line but also to not break down thereby changing its dielectric constant. The key characteristics required for such fluid use are:

1. High oxidation stability:
  - a. long life and protection;
  - b. no oxidation materials; and
  - c. no changes in chemical properties.
2. Viscosity Characteristics:
  - a. low pour point for cold temperature service, particularly in cold temperature regions; and
  - b. high Viscosity Index for best viscosity under various operating temperatures.
3. Corrosion Inhibition Properties:
  - a. inhibits contaminants in the fluid;
  - b. inhibits water;
  - c. inhibits oxidation by-products; and
  - d. inhibits changes in the fatty acids (in the case of vegetable oils).
4. Seal, Polymer, Resin Compatibility:
  - a. with old and new seal materials; and
  - b. with resin and other insulating materials.

Another demand placed upon electrically-insulating fluid is the requirement that it maintain a certain degree of stability in terms of insulating properties despite some of the physical and chemical changes that take place during extended use.

Therefore, it is a primary object of the present invention to present a composition and method which improve over and/or solves the problems and deficiencies in the art. Further objects of the invention include the provision of a vegetable oil-based composition and method which:

- a. can be substituted for existing electrically-insulating fluids used in such electrical components as transformers and fluid-filled transmission lines, but is more environmentally-friendly and less toxic;
- b. is more biodegradable than petroleum-based or some synthetic-based fluids;
- c. has a renewable source;
- d. meets the specifications and requirements typically recognized by the industry for such fluids and/or performs generally equivalently to existing fluids;
- e. is relatively long-lasting and durable over a variety of operational and environmental conditions; and
- f. is economical to make, use, and maintain.

These and other objects, features, and advantages of the present invention will become more apparent with reference to the accompanying specification and claims.

## SUMMARY OF THE INVENTION

The present invention relates to a vegetable oil-based electrically-insulating fluid for use in electrical components that need such a fluid, such as for example, electrical transformers and fluid-filled electrical transmission cables or lines. A base oil made from vegetable oil, especially soybean and/or corn oil, is chemically modified by at least partial hydrogenation. To achieve this result, the base oil is optimized, through the process of hydrogenation, to produce maximum possible stability of the vegetable oil. This process is necessary for transformer equipment and transmission line applications. An antioxidant may be added to the base oil.

The vegetable-based oil of the present invention can be further processed with the additional step of winterization to remove crystallized fats and improve the pour point of the base oil without the necessity of heating the oil. An additive package for the present invention can be included which contains materials specifically designed for improving the properties of vegetable oil for this application.

The combination of the processed vegetable oil and additives produces an electrically-insulating fluid that withstands the rigors of field use involving a wide range of temperatures.

According to the invention, an electrical component containing the vegetable-based oil described above is set forth. The vegetable-based oil, contrary to existing petroleum-based or synthetic oils, is biodegradable and, therefore, safer to the environment and to living things. It also is based on a natural, renewable resource.

## BRIEF DESCRIPTION OF THE DRAWINGS

FIG. 1 is a graph illustrating the Active Oxygen Method as a means of expressing stability of vegetable oils.

FIG. 2 is a graph illustrating biodegradation of partially hydrogenated and winterized soybean oil before and after long term exposure to high pressure and high temperature in hydraulic pump tests.

## DESCRIPTION OF THE PREFERRED EMBODIMENTS OF THE INVENTION

To assist in a better understanding of the invention, preferred embodiments of the present invention will be described below in detail. Examples will be set forth. To give concrete examples, the embodiments are discussed in the context of fluid used as the electrically-insulating/cooling fluid in electrical transformers (electric utility transmission, power, and distribution transformers) and fluid-filled electrical transmission cables or lines, such as are known in the art. This is not by way of limitation to the invention.

An electrically-insulating fluid for transformers comprises crude vegetable oil, especially soybean and/or corn oil, made from commodity grains which have been partially hydrogenated and winterized combined with a thinning ester and antioxidant(s) to produce a fluid having a kinematic viscosity in the range of 20–40 cSt at 40° C. The hydrogenated vegetable oil comprises less than 95% by weight of the fluid, and the fatty acid profile of the resulting electrically-insulating fluid includes C24:0. The resulting oil has a viscosity preferably in the range of 25–50 cSt at 40° C. vs. prior art soybean-based oils which are high viscosity functional lubricants having viscosity ranges of 2,000–2,500 cSt at 25° C.

Vegetable oil-based electrically-insulating fluids, specifically soybean oil-based or corn oil-based fluids, according to

the preferred embodiments of the invention were tested under exacting laboratory conditions and in field use. The analysis of soybean oil-based electrically-insulating fluid revealed two primary findings. First, the dielectric qualities associated with the fluid were comparable to those qualities associated with other vegetable oil-based fluids or petroleum-based fluids. Second, durability of the fluid was generally a consistent problem with and without the combination of various additives.

In addressing the issue of durability, it was determined that partially hydrogenated soybean oil presented optimal results in bench tests and with field results. Since the demands on the product called for its use in outdoor conditions, the soybean oil was winterized to aid its low temperature utility. The winterized, at least partially hydrogenated soybean oil was found to have superior characteristics both in durability and in dielectric property.

Another problem with the soybean oil was its naturally higher than desired viscosity, which was modified with the addition of soybean-based esters to develop the desired viscosity.

A myriad of additive products were tested in the analysis of soybean oil-based electrically-insulating fluids. The various bench tests and outdoor field tests performed on the alternative combinations of additives and soybean oils yielded a wide variety of data. The bench tests provided comparative data in the areas of viscosity, density, pour point, flash point, and acid value. The testing is discussed more fully below.

The process of hydrogenating soybean oil made from commodity soybeans is well known in the art. It is explained in the following reference: *Handbook of Soy Oil Processing and Utilization* (Editors: D R. Erickson, E H. Pryde, O. L. Brekke, T. L. Mountsk R. A. Falb), published by American Soybean Association and American Oil Chemists' Society, Copyright 1980, Third Printing 1985; see, for example, *Hydrogenation Practices*, Chapter 9; and *Partially Hydrogenated-Winterized Soybean Oil*, Chapter 12. This is incorporated by reference herein.

The amount of hydrogenation can vary. However, the amount can be such that the hydrogenation is about that of what is known in the art as maintaining liquidity of soybean oil (salad quality oil). This is a standard term in the art. The hydrogenation, as will be discussed further below, could alternatively be described as having an Iodine Value in the range of 100–120. This is a well-known test for amount of hydrogenation. The step of partial hydrogenation is used because it saturates the fatty acid chains, thereby raising the oleic content of commodity soybean oil significantly. For example, conventional commodity soybean oil available from any number of sources generally has an oleic acid content of about 20%. Partial hydrogenation increases this to around 40%. Thus, this approaches the much higher natural oleic acid contents of such oils as rapeseed and canola.

Still further, it is better for the electrically-insulating fluid to have a linolenic acid amount as low as possible. Conventional commodity soybean oil has a linolenic content of around 8%. Partial hydrogenation reduces this to around 3%.

Winterization is also a well-known processing step to those in the art. See also *Handbook of Soy Oil Processing and Utilization*, referenced above and incorporated by reference herein. Winterization is an optional step. It is useful in particular with electrically-insulating fluids that will be used outside in extreme temperatures. The winterization can be so that the fluid does not react adversely down to lower temperatures. With addition of pour point depressants, temperatures as low as  $-25^{\circ}\text{C}$ . can be obtained.

The thinning esters are also optional. They are beneficial because they allow the fluid to be customized for different needs of different users. Some users want or need an electrical insulating fluid with a lower viscosity. Others need a higher viscosity. The thinning esters can be methyl esters derived from soybeans or other grains. Therefore, they too would be biodegradable. The range of carbon chain length for such thinning esters can be preferably in the range of 16 to 18, if using a natural product. Other chain lengths will work. Those skilled in the art would be able to determine which methyl esters or other thinning agents would work and how much is needed for a certain application. Alternatives would be methyl esters derived from palm oil and coconut oil, for example, and perhaps alcohol. Alcohol may increase flash point, which is to be avoided because of the high temperatures that may be experienced in applications of the present invention.

An additive to the base partially hydrogenated oil is an antioxidant. This increases the durability and longevity of the fluid over the conditions experienced in a transformer or transmission line or analogous uses. The antioxidant used is preferably tertiary butylhydroquinone (TBHQ). Others are possible. The essential characteristic of the antioxidant used is that its working mechanism is a free radical scavenger. It is believed that most, if not all, antioxidants used as food preservatives or associated with food uses would work. Additional antioxidants can also be added. Here a quantity of citric acid was added. Still further, tocopherols were added, which are from soybeans, but are many times lost through soybean processing.

If the base oil has a hydrogenation level or oleic acid level that is high enough, an antioxidant may not be required for durability and longevity over the life of a given electrical component. One of ordinary skill in the art would be able to determine whether an antioxidant is required for a specific vegetable oil in a specific application by routine experimentation.

An alternative to using at least partially hydrogenated soybean oil for the base oil according to the invention would be to use soybean oil from genetically-engineered (or specially bred) soybeans that are high in oleic acid. Soybean oil made from such soybeans can be purchased from DuPont and Pioneer Hi-Bred International. Such soybeans are believed to have an oleic acid content at least on the order of 40%. They also are believed to have a linolenic acid content on the order of 3%.

Of the fatty acids in the composition of soybean oil, oleic acid is the most important relative to use of such oil as an electrically-insulating fluid. The higher the oleic acid content the better. It has been found that the lower the linolenic content, the better also. Of course, if the oleic content is raised, other acids must be reduced, and this can occur for lowered linolenic acid when oleic is raised.

## EXAMPLES

### Example 1

#### Oxidation of Oils

##### 60 Test Results

Soybean oil in its natural form is oxidatively unstable, and when used in a transformer and transmission line system, it thickens up. In extreme cases, the oil, if left in the system, will polymerize. The most common way to determine oxidative stability of vegetable oils has been the Active Oxygen Method (AOM). Recently, however, another method has been introduced using what is called the oxidative stability

instrument (OSI). FIG. 1 of the drawings and Table 1 following show an example of data presented in the literature using each of these methods:

TABLE 1

| Oxidative stability instrument (OSI) used in determining oxidation of canola and partially hydrogenated soybean oil (ABIL conducted tests). |                 |          |
|---------------------------------------------------------------------------------------------------------------------------------------------|-----------------|----------|
| Oil Type                                                                                                                                    | Viscosity (cSt) | OSI Time |
| Canola w/Antioxidant                                                                                                                        | 38.77           | 39.18    |
| Canola w/o Antioxidant                                                                                                                      | 38.70           | 9.04     |
| Chemically-Modified Soy Oil w/ Antioxidant                                                                                                  | 38.45           | 50.70    |
| Chemically Modified Soy Oil w/o Antioxidant                                                                                                 | 36.47           | 31.30    |

It can be seen that the chemically-modified soy oil with antioxidant, according to the invention, has a viscosity on the order of canola oil with antioxidant.

## Example 2

## Pump Tests

5

A better but more expensive method to investigate stability of vegetable oils in industrial application, such as transformer and transmission line cooling systems, is the use of the ASTM D2271 hydraulic pump test. This is a time consuming (1000-hour) test which helps determine both the pump wear protection property as well as the stability of the test oil. In this test, the stability of the test oil is determined by changes in its viscosity during the test. An oil that maintains its viscosity (changes little), after completion of this test, will perform better in long-term use in electrical transformers and electrical fluid-filled transmission lines.

Thousands of hours of bench testing of treated and untreated soybean oils and other vegetable oils have been performed. Table 2 shows a comparison of selected vegetable oils including a number of soybean oils as tested in the ASTM D2271 test at the University of Northern Iowa College of Natural Sciences, Ag-Based Industrial Lubricant (ABIL) research facility at 400 Technology Place, Waverly, Iowa 50677.

TABLE 2

| Using ASTM D2271, 1000-hour at 79° C. pump tests, the stability of various vegetable oils were compared to determine suitability of soybean oil regarding stability. |  |  |  |  |
|----------------------------------------------------------------------------------------------------------------------------------------------------------------------|--|--|--|--|
|----------------------------------------------------------------------------------------------------------------------------------------------------------------------|--|--|--|--|

| Item | Oil Type/                             | Viscosity |             |         |       |          |
|------|---------------------------------------|-----------|-------------|---------|-------|----------|
|      |                                       | #         | Description | Initial | Final | % Change |
| 1    | Palm Oil                              | 41.78     | 54.75       | 31.0    |       |          |
| 2    | Cotton Oil                            | 37.94     | 56.23       | 48.2    |       |          |
| 3    | High Oleic Canola Oil (1)             | 38.20     | 57.73       | 51.1    |       |          |
| 4    | High Oleic Canola Oil (2)             | 39.50     | 56.70       | 43.5    |       |          |
| 5    | High Oleic Sunflower Oil              | 37.83     | 53.87       | 42.4    |       |          |
| 6    | Ultra High Oleic Sunflower Oil        | 40.46     | 56.69       | 40.1    |       |          |
| 7    | Crude Soy Oil (hexane extracted)      | 29.91     | 73.77       | 146.6   |       |          |
| 8    | Crude Soybean Oil (expelled)          | 30.16     | 65.87       | 118.4   |       |          |
| 9    | Crude Soybean Oil (extruded/expelled) | 30.93     | 65.18       | 110.7   |       |          |

TABLE 2-continued

Using ASTM D2271, 1000-hour at 79° C. pump tests, the stability of various vegetable oils were compared to determine suitability of soybean oil regarding stability.

| Item | Oil Type/                                      | Viscosity |             |         |       |          |
|------|------------------------------------------------|-----------|-------------|---------|-------|----------|
|      |                                                | #         | Description | Initial | Final | % Change |
| 10   | Low Linolenic Crude Soybean Oil                | 31.33     | 70.89       | 126.3   |       |          |
| 11   | Bleached Soybean Oil (ASTM 2882-100 hr test)   | 29.63     | 31.65       | 6.8*    |       |          |
| 12   | Refined Soybean Oil (ASTM 2882-100 hr test)    | 29.72     | 31.99       | 7.6*    |       |          |
| 15   | Deodorized Soybean Oil (ASTM 2882-100 hr test) | 29.59     | 31.34       | 5.9*    |       |          |

\*Note:

Items 11-13 were in a different ASTM test using a higher pressure setting (2000 psi) but a shorter test of 100 hrs and a temperature of 65° C.

## Example 3

## Modified Oil and Fluid Selection

30 Next, effort was focused on chemical modification of soybean oil as a means of increasing its oxidative stability. This led to the identification of one of the most stable, commercially-available, chemically-modified soybean oils. This oil is a soybean oil which is partially hydrogenated.

35 When combined with two antioxidants, citric acid and tertiary butylhydroquinone (TBHQ), the oil was significantly more stable than other soybean oils. In the preferred embodiment, the level of TBHQ was in the range of 200–10,000 parts/million (ppm), and the level of citric acid ranged from 10–1,000 ppm.

40 Furthermore, the oil was winterized in order to improve its pour point in cold temperatures. Table 3 shows the 45 performance results of the selected oil (henceforth, the “base oil”) in the ASTM 2271 test. When compared with test oil (item #8, Table 2), the chemically-modified soybean oil showed almost 50% improvement in its viscosity stability. The OSI results of the same oil were shown in Table 1, 50 previously.

TABLE 3

| Item | Oil Type/                                  | The selected soybean oil for transformer and transmission line cooling oil. |             |           |       |          |
|------|--------------------------------------------|-----------------------------------------------------------------------------|-------------|-----------|-------|----------|
|      |                                            | #                                                                           | Description | Viscosity |       |          |
|      |                                            |                                                                             |             | Initial   | Final | % Change |
| 60   | Chemically-Modified Soybean Oil (base oil) | 18                                                                          | 38.62       | 56.45     | 46.2  |          |

65 Once the optimal base oil was identified, it was blended with various additive components and/or packages and tested for dielectric breakdown voltage using ASTM 877-87

test method Dielectric Breakdown Voltage on Insulating Liquids Using Disk Electrodes. The purpose was to determine the breakdown voltage for each oil; preliminary results are shown in Table 4.

TABLE 4

| Oil Type                                                         | Dielectric Breakdown Voltage (kV) |
|------------------------------------------------------------------|-----------------------------------|
| Crude Untreated Soybean Oil                                      | 6.30                              |
| Crude Soybean Oil +                                              | 10.60                             |
| Antioxidants                                                     |                                   |
| Crude Soybean Oil with 20% Thinning Methyl Esters                | 11.75                             |
| Crude Soybean Oil with 20% Thinning Methyl Esters + Antioxidants | 16.20                             |
| Modified* Soybean Oil                                            | 16.89                             |
| Modified* Soybean Oil + 20% Thinning Methyl Esters               | 14.25                             |
| Modified* + 20% Thinning Methyl Esters + Antioxidants            | 19.20                             |
| Modified* + Antioxidants                                         | 23.95                             |

\*Modified: chemically-modified (partially hydrogenated) and winterized.

Table 4 shows preliminary results which are useful for non-quantitative comparative purposes. Table 5, which appears below, contains current results of breakdown voltage achieved with the fluid of the present invention.

The inclusion of methyl esters had to be with consideration to compatibility of soybean oil and methyl esters with seals and other elastomers used in transformers and transmission line cooling systems. Rubber compatibility tests, requiring immersion of elastomer materials in test fluid for 72 hours at 100° C. and measurement of expansion of the material, indicated that the base oil had under 5% expansion, while the thinning methyl ester fluid (when tested alone) had expansion as high as 46%. The blends identified present suitable dielectric values with under 10% expansion in elastomer compatibility tests.

The base oil, according to the preferred embodiment, presents the following characteristics:

#### Characteristics:

|                 |                                                       |
|-----------------|-------------------------------------------------------|
| Appearance      | Clear and brilliant at room temperature (observation) |
| Color           | 1.0 red maximum (AOCS Cc 13b-45)                      |
| Peroxide Value  | 1.00 meq/kg maximum (AOCS Cd 8-53)                    |
| Flavor and Odor | Bland (sensory evaluation)                            |
| Iodine Value    | 100-120                                               |

#### chemical (Fatty Acid) Composition:

|           |          |
|-----------|----------|
| Palmitic  | 7.4-10.2 |
| Stearic   | 4.3-6.2  |
| Oleic     | 35-48    |
| Linoleic  | 34-54    |
| Linolenic | 3.5-8    |

The combination of the additive components with the specially-prepared soybean oil blended with thinning esters resulted in a synergy that is not common in other vegetable oils of unsaturated nature, such as soybean oil. The recog-

nition of this synergy combined with an understanding that established test methods (used in literature) do not measure true performance of the vegetable oils in transformer and transmission line cooling system were essential in the development of this product. The established methods of evaluating the performance of electrically-insulating fluid are designed for petroleum-based products and are not always indicative of true performance of the vegetable oil-based products.

#### Example 4

#### Field Tests and Blending

Once the finished product was identified, it was used for field tests involving the facilities and transformer components of Waverly Light and Power, 1002 Adams Parkway, Waverly, Iowa 50677. Additionally, the oil, when tested mechanically in a blended state 50/50 with petroleum-based oil, showed similar stability performance. Test results indicated there was almost no difference in the change of viscosity in the test fluids during the comparative mechanical testing.

Some of our field test transformers have over two years of service on them, utilizing the BioTrans™ fluid of the present invention. Samples of fluid were taken and tested in accordance with ASTM D 877 and ASTM D 445. The following Tables 5 and 6 are testing results (similar to Tables 3 and 4 above) for specific field tested fluids according to the present invention.

TABLE 5

| Dielectric Breakdown in accordance with ASTM D 877.                    |                        |
|------------------------------------------------------------------------|------------------------|
| ID #                                                                   | Breakdown Voltage (kv) |
| BioTrans™ (new, unused chemically modified soybean oil + antioxidants) | 44.5                   |
| Sample 1                                                               | 44.34                  |
| Sample 2                                                               | 43.98                  |
| Sample 3                                                               | 41.56                  |
| Sample 4                                                               | 40.16                  |

TABLE 6

| Viscosity in accordance with ASTM D 445.                               |                 |
|------------------------------------------------------------------------|-----------------|
| ID #                                                                   | Viscosity (cSt) |
| BioTrans™ (new, unused chemically modified soybean oil + antioxidants) | 37.38           |
| Sample 1                                                               | 35.58           |
| Sample 2                                                               | 37.25           |
| Sample 3                                                               | 35.08           |
| Sample 4                                                               | 35.44           |

TABLE 7

| Field testing results for commodity soy oil chemically modified. Samples visually appeared as the oil did when originally placed into service. |            |       |          |       |               |       |            |       |          |
|------------------------------------------------------------------------------------------------------------------------------------------------|------------|-------|----------|-------|---------------|-------|------------|-------|----------|
|                                                                                                                                                | Sample 1   |       | Sample 2 |       | Sample 3      |       | Sample 4   |       | Sample 5 |
| Test date                                                                                                                                      | 6/99       | 5/00  | 6/99     | 5/00  | 6/99          | 5/00  | 6/99       | 5/00  | 5/00     |
| Hours                                                                                                                                          | 12400      | 20656 | 7200     | 15456 | 11040         | 19296 | 12499      | 20656 | 7032     |
| Antiox. (AO)                                                                                                                                   | TBHQ       |       | TBHQ     |       | TBHQ          |       | TBHQ       |       | TBHQ     |
| AO%                                                                                                                                            | 0.5        |       | 0.5      |       | 0.5           |       | 0.5        |       | 0.5      |
| Dielectric value                                                                                                                               | 44.34      | 46.07 | 43.98    | 43.8  | 41.56         | 48.57 | 40.16      | 44.07 | 41.43    |
| OSI                                                                                                                                            | 7.02       |       | 57.6     | 47.58 | 47.87         | 85.1  | 11.4       | 11.58 | 46.68    |
| Viscosity                                                                                                                                      | 35.61      | 35.64 | 37.25    | 37.35 | 36.05         | 37.04 | 35.45      | 35.61 | 37.34    |
| Installation                                                                                                                                   | 4/98 retro |       | 8/98 new |       | 6/98 retro    |       | 4/98 retro |       | 8/98 new |
| Customers                                                                                                                                      | 7          |       | 1        |       | Street lights |       | 5          |       | 1        |
| KVA                                                                                                                                            | 25.00      |       | 10.00    |       | 1.00          |       | 25.00      |       | 10.00    |

Viscosity has stabilized, so the oil has maintained its resistance to flow characteristics and is neither thickening or thinning.

OSI values are remaining consistent with little oxidation occurring since 6/11/99.

Dielectric values are within the 40–50 kV range. According to our test results, the dielectric fluid appears to be in very good condition.

The tests with the blended soybean-based oil and petroleum oil established that it is possible to retrofit the base oil according to the present invention into existing electrical transformers or transmission lines. Even if some petroleum-based oil remains after draining, it appears that it will have no affect on operation after it is refilled with the vegetable-based oil of the present invention.

At the conclusion of the various comparative analyses, it was determined that the combination of the chemical modification of the vegetable oil and the addition of vegetable-based esters and other chemical property enhancers provided superior results over the unmodified soybean oil or other vegetable oils. Use of the thinning esters with some of the antioxidants provided a synergy with the soybean oil, which enhanced the durability of the fluid far beyond what the existing arts indicated. Additionally, the additives produced positive results in the areas not directly related to the performance of the oil but to its environmental benefits, such as biodegradability and toxicity.

#### Example 5

##### Biodegradability

Additional testing of the oil included biodegradability tests to determine the biodegradation of the mixture (fresh and after use in 1000-hour hydraulic pump test) in soil using CO<sub>2</sub> evolution in a given number of days. FIG. 2 shows the results of these tests, namely biodegradation of partially hydrogenated soy oil with 200 ppm TBHQ measured as CO<sub>2</sub> production.

#### Example 6

##### Fire/Flash point

Another aspect of the present invention is the fluid's inherent high flash point/fire point. By "high flash point" it is meant that the oil has been shown to have relatively high flash point characteristics compared to conventional petroleum or mineral oil-based fluids. It can, therefore, be used in applications that either require or desire a higher flash point. Fire resistant (higher flash point) fluids are used to increase

the fire safety of such things as transformers and fluid-filled switches primarily for those electrical devices located within or near buildings. Many times the use of fire resistant fluids is required by specifications for new building construction, by insurance companies or attorneys for existing buildings, or during building remodeling. Changed codes or proximity to public access spaces may dictate a fire resistant fluid be used.

Fire resistant fluids in use typically have a fire point of 300° C. or higher per National Electrical Code. Regular petroleum-based fluids for transformer use have fire points in the 140° C. range. Present fire resistant fluids are either petroleum-based or are made from synthetic fluids, like silicone. All are hydrocarbon-based and are minimally biodegradable.

Fluid according to the present invention, therefore, is "fire resistant" in electrical components. "Fire resistant" would encompass all blends of the fluid that have a fire point rating of 300° C. or better. The results of an open cup flash and fire point for the oil of the present invention are shown in Table 8.

TABLE 8

| Flash/Fire Point test results for chemically-modified soybean oil. |                                     |                                    |
|--------------------------------------------------------------------|-------------------------------------|------------------------------------|
| Sample                                                             | Flash Point<br>ASTM D92 (° C./° F.) | Fire Point<br>ASTM D92 (° C./° F.) |
| Chemically Modified Soybean Oil                                    | 328° C./635° F.                     | 342° C./646° F.                    |

The tests were performed according to ASTM D92 protocol. It can be seen that the oil has a flash point and a fire point well over 300° C.

#### Example 7

##### Corn Oil

Since corn oil was expected to behave similarly to soybean oil, it was tested. The results are shown in Table 9.

TABLE 9

Testing results for corn oil.

| ASTM  | Parameter                      | AN991<br>Soybean oil<br>(non-genetically<br>engineered) | AN500-C<br>corn oil | ASTM D3487<br>minimums for<br>mineral<br>transformer oils |
|-------|--------------------------------|---------------------------------------------------------|---------------------|-----------------------------------------------------------|
| D1533 | Moisture (ppm)                 | 93                                                      | 70                  | 35 max.                                                   |
| D971  | Interfacial tension (dynes/cm) | 21.7                                                    | 22.8                | 40 min.                                                   |
| D974  | Acid number (mg KOH/g)         | 0.080                                                   | 0.069               | 0.03 max.                                                 |
| D1500 | Color number                   | <1.0                                                    | <1.5                | 0.5 max.                                                  |
| D1524 | Visual examination             | Clear with part.                                        | Clear with part.    | Clear & bright                                            |
| D877  | Dielectric BV (kV)             | 44                                                      | 50                  | 30 min.                                                   |
| D1816 | Dielectric BV (kV)             | 22                                                      | 26                  | 28 min.                                                   |
| D924  | Power factor (% at 25° C.)     | 17.0                                                    | 17.0                | 0.05 max.                                                 |
| D924  | Power factor (% at 100° C.)    | 5.0                                                     | 15.3                | 0.30 max.                                                 |
| D2668 | Oxidation inhibitor (%)        | 0.315                                                   | 0.429               | 0.3 max.                                                  |
| D129  | Specific gravity               | 0.916                                                   | 0.920               | 0.91 max.                                                 |
| D88   | Viscosity (SUS)                | 193                                                     | 155                 | 66 max.                                                   |
| D97   | Pour point (°C.)               | 15                                                      | 15                  | -40 max.                                                  |
| D92   | Flash point (°C.)              | 310                                                     | 321                 | 145 min.                                                  |
| D92   | Fire point (°C.)               | 360                                                     | 349                 |                                                           |
| D1807 | Refractive index               | 1.4705                                                  | 1.4718              |                                                           |
| D1275 | Corrosive sulfur               | Noncorr.                                                | Noncorr.            | Noncorr.                                                  |

From the foregoing information and examples, it will be evident that the invention provides an improved non-petroleum-based, environmentally safe electrically-insulating fluid that can be commercially used in such components as transformers and transmission lines. The electrically-insulating fluid of the invention utilizes vegetable oil which comprises less than 95% by weight of the fluid. The additive package used in the preferred embodiment contains materials specifically designed for transformer cooling applications. The combination of the specific vegetable oil and the additive(s) has produced an electrically-insulating fluid that withstands the rigors of field use involving a wide range of temperatures. The preparation of the vegetable oil-based electrically-insulating fluid of the invention does not involve any heating with an outside heating source. Furthermore, the electrically-insulating fluid of the invention has been designed to maintain a stable viscosity at a lower range of viscosity than those designed for possible use with other vegetable oils. The soybean oil-based electrically-insulating fluid of these examples is produced using an additional step of winterization to remove crystallized fats and improve the pour point of the base oil.

It is believed that there may be, at times, condensation inside large electrical transformers, even though they are encased in metal and sealed. It is to be understood that other additives could be included with the electrically-insulating fluid described herein to address further matters that may occur with such fluids. For example, an anti-sludge substance, such as is known in the art, could be added to combat any condensation. Also, an anti-foaming agent can be added to reduce foaming under vacuum. Another example is an anti-corrosion substance to deter acid interaction. These products are all available "off the shelf", and the amounts to be added are well within the knowledge of those of ordinary skill in the art.

The relative amounts of the various components of the composition described herein can vary. If the composition includes just base vegetable oil (partially hydrogenated or made from high oleic content grain) and the antioxidant TBHQ, the ratio could be (by weight) from 99.98% base soybean oil and 0.02% TBHQ to 99% base vegetable oil and 1% TBHQ. The preferred ratio is 99.5% base vegetable oil and 0.5% TBHQ.

If a second antioxidant is added, such as citric acid, the ranges could be from 99.97% base vegetable oil: 0.02% TBHQ: 0.01% citric acid to 98.99% base vegetable oil: 1% TBHQ: 0.01% citric acid.

If thinning esters are utilized, they can comprise on the order of 0%-30% by weight of the fluid (depending upon desired viscosity) and alter the percentages of the base oil and antioxidants accordingly.

The method of making the fluid comprises processing commodity soybeans, or other grains, in conventional manners to produce vegetable oil. The oil is partially hydrogenated to a form similar to "salad quality oil" and winterized, both by known in the art methods. An antioxidant or multiple antioxidants can be added to the base oil by mixing it in by known methods. A thinning ester can be blended in by known methods. The proportions can be such as are within the ranges expressed above. Alternatively, the beginning oil could be high oleic acid content vegetable (soybean and/or corn) oil which are genetically altered, or specially bred. Hydrogenation may not be required if the oleic content is high enough. Winterization could still be performed and the antioxidant(s) mixed in. Thinning esters could be used to the extent needed or desired.

Electrical components, such as large transformers or fluid-filled transmission lines, such as are known in the art, can be constructed by building the component with a cavity or space(s) to hold an electrically-insulating fluid. A fluid of the type described above could then be placed in the cavity or space.

Pour stabilizers for vegetable oils are available off-the-shelf from a variety of vendors and manufacturers. Examples are Viscoplex® materials marketed by Rohmax Additives GmbH, Kirschenallee, D-64293 Darmstadt, Telephone +49 6151 18-09. Specific examples are Viscoplex® 10-310 and 10-930. One form of product Viscoplex® 10-310 is a ester/rapeseed oil solution of a polymer on the bias of long-chain methacrylic acid esters and has the chemical name diethylhexyl adipate, CAS number 103-23-1, concentration 5-10%. These products effectively lower the pour point and stabilize the pour point to at least -25° C., and, thus, provide storage stability even under severe conditions. A typical addition rate is 0.5% wt. for a storage

stability at  $-25^{\circ}\text{ C}$ . It is biodegradable. Another form of product Viscoplex® 10-310 is a solution of polyalkyl methacrylate (PAMA) in a biodegradable carrier oil.

As is well known in the art, an antioxidant is defined as an organic compound added to rubber, natural fats and oils, food products, gasoline and lubricating oils to retard oxidation, deterioration, and rancidity. Rubber antioxidants are commonly of an aromatic amine type, such as di-beta-naphthyl-para-phenylenediamine and phenyl-beta-naphthylamine; a fraction of a percent affords adequate protection. The National Rubber Producers' Research Association has developed a technique for adding to a rubber mix organo-nitrogen compounds that are converted during vulcanization to a powerful antioxidant that becomes part of the rubber molecule, making it impossible to wash out. Many antioxidants are substituted phenolic compounds (e.g., butylated hydroxyanisole, di-tert-butyl-para-cresol, and propyl gallate). Food antioxidants are effective in very low concentrations (not more than 0.01% in animal fats) and not only retard rancidity but protect the nutritional value by minimizing the breakdown of vitamins and essential fatty acids. Sequestering agents, such as citric and phosphoric acids, are frequently employed in antioxidant mixtures to nullify the harmful effect of traces of metallic impurities. Note: Maximum concentration of food antioxidants approved by FDA is 0.02%.

Examples of other antioxidants are:

2,6, -di-tert-butyl-methylphenol;  
2,4-dimethyl-6-tert-butylphenol;  
N,N'-di-sec-butyl-para-phenylenediamine;  
low-ash dioctyl diphenylamine;  
N,N'-di-isopropyl-para-phenylenediamine;  
high molecular weight hindered phenolic antioxidant;  
N,N'-bis-(1,4-dimethylpentyl)-para-phenylenediamine;  
high molecular weight, phenolic type antioxidant for  
polypropylene;  
Antioxidant B™;  
Antioxidant D™;  
butylated hydroxyanisole;  
butylated hydroxytoluene;  
maleic acid BP (cis-Butenedioic acid  $\text{C}_4\text{H}_4\text{O}_4$  9116.07);  
taxilic acid;  
tocopherols (whether natural (some can occur in  
soybeans), genetically enhanced or produced (e.g.,  
in soybeans), or added).

Others are possible that function similarly with the base oil described herein.

The fluid according to the present invention can be used in new equipment, as well as retrofilling existing equipment. An option is to include a blend of generic petroleum-based or synthetic-based oils with the fluid according to the present invention, or simply a blend with pure mineral oil. Another option is to blend the fluid according to the present invention with standard mineral oil to the exact point where a fire point of  $300^{\circ}\text{ C}$ . is reached to produce either a higher fire point fluid. The advantages of such a fluid include improved pour point, improved stability, and lower price. Retrofilling and/or blending also makes an existing fluid more environmentally friendly.

Therefore, embodiments of the invention include the fluid according to the invention alone or in blends with any of the following:

petroleum-based fluids including generic transformer oils; synthetic fluids, like silicone; and pure mineral oil.

One of skill in the art would be able to determine other fluids with which the present invention could be blended/mixed. It is further emphasized that the fluid according to the present invention is compatible with mineral oil, petroleum, or synthetic dielectric fluids. Therefore, there is no problem blending nor any problem in retrofilling.

Transformers originally filled with conventional transformer oil can be retrofilled with a fire-resistant oil to increase the fire safety margin of these units or environmentally friendly fluid to decrease environmental effects. One of ordinary skill in the art can determine how to retrofill an electrical component. An example procedure can be found at [www.electricityforum.com/et/May96/trans.htm](http://www.electricityforum.com/et/May96/trans.htm).

It is to be understood that the fluid according to the present invention is believed to be useful in all applications where electrical devices require fluid for insulating or dielectric properties. Additional examples include oil-filled electrical switches, oil-filled electrical bushings, oil-filled capacitors, oil-cooled reactors, and oil-filled electrical regulators.

Having thus described the invention in connection with the preferred embodiments thereof, it will be evident to those skilled in the art that various modifications can be made to the preferred embodiments described herein without departing from the spirit and scope of the invention. It is our intention, however, that all such modifications that are evident to those skilled in the art will be included within the scope of the following claims.

What is claimed:

1. An insulating fluid for electrical components comprising:  
an amount of oil comprising  
a base oil selected from the group consisting of at least  
partially hydrogenated vegetable oil, vegetable oil  
higher in oleic acid content relative to a corresponding  
vegetable oil made from commodity grain, and  
combinations thereof, the vegetable oil selected from  
the group consisting of soybean oil, corn oil, and  
combinations thereof, wherein the vegetable oil is  
corn oil made from corn which is higher in oleic acid  
content compared to commodity corn and wherein  
the corn is genetically-modified or bred;  
and an antioxidant.
2. A fluid of claim 1 wherein the base oil comprises  
detectable to less than one hundred percent of the fluid.
3. The fluid of claim 1 wherein the antioxidant comprises  
between 200 to 10,000 ppm of the fluid.
4. The fluid of claim 3 wherein the antioxidant produces  
an electrically-insulating fluid having a kinematic viscosity  
in the range of 20-40 cSt as desired at  $40^{\circ}\text{ C}$ . and the  
antioxidant is a free radical scavenger.
5. The fluid of claim 1 wherein the base oil is winterized.
6. The fluid of claim 1 wherein the oleic acid content of  
the oil is about 30% or greater.
7. The fluid of claim 1 wherein the linolenic acid content  
of the oil is about 5% or less.
8. The fluid of claim 1 wherein the antioxidant is tertiary  
butylhydroquinone.
9. The fluid of claim 8 wherein the tertiary butylhydro-  
quinone comprises between 200 ppm and 10,000 ppm of the  
fluid.
10. The fluid of claim 1 comprising two antioxidants.
11. The fluid of claim 8 further comprising citric acid.
12. The fluid of claim 11 wherein the citric acid comprises  
in the range of 10 to 1000 ppm and the tertiary butylhy-  
droquinone comprises in the range of 200 to 10,000 ppm.

13. The fluid of claim 1 further comprising a thinning agent.

14. The fluid of claim 13 wherein the thinning agent comprises thinning esters.

15. The fluid of claim 14 wherein the thinning esters comprise methyl esters in the range of carbon chain lengths of 16 to 18.

16. The fluid of claim 15 wherein the methyl esters comprise approximately 0% to 30% by weight of the fluid based on desired viscosity.

17. A method of making an electrical component comprising:

creating an electrically-insulating fluid comprising a base oil selected from the group consisting of at least partially hydrogenated vegetable oil, vegetable oil higher in oleic acid content relative to a corresponding vegetable oil made from commodity grain, and combinations thereof, wherein the vegetable oil is corn oil made from corn which is higher in oleic acid content compared to commodity corn and wherein the corn is genetically-modified or bred.

18. The method of claim 17 wherein the fluid further comprises an antioxidant.

19. The method of claim 17 wherein the base oil comprises detectable to less than one hundred percent of the fluid.

20. The method of claim 17 wherein the electrical component is an electrical transformer.

21. The method of claim 20 wherein the electrical transformer is a electric utility transmission and distribution transformer.

22. The method of claim 17 wherein the electrical component is a fluid-filled electrical transmission cable.

23. The method of claim 17 wherein the base oil is replaced into the electrical component after draining it of petroleum-based oil.

24. The method of claim 18 wherein the antioxidant comprises from 0.02% to 1.0% by weight of the fluid.

25. The method of claim 17 wherein the base oil is winterized.

26. The method of claim 17 wherein the viscosity of the fluid is adjusted by blending a thinning substance into the fluid.

27. An electrical component comprising a body, the body including a cavity for a fluid; and an electrically-insulating fluid in the cavity comprising a base oil from the group consisting of at least partially hydrogenated vegetable oil, vegetable oil higher in oleic acid content relative to a corresponding vegetable oil made from commodity grain, and combinations thereof, wherein the vegetable oil is corn oil which is higher in oleic acid content compared to commodity corn and wherein the corn is genetically-modified or bred.

28. The component of claim 27 wherein the fluid further comprises an antioxidant.

29. A component claim 27 wherein the base oil comprises detectable to less than one hundred percent of the fluid.

30. The component of claim 27 wherein the component comprises an electrical transformer.

31. The component of claim 27 wherein the component comprises a fluid-filled electrical transmission cable.

32. The component of claim 27 wherein the fluid is winterized and has a kinematic viscosity in the range of 20-40 cSt at 40° C.

33. The component of claim 27 wherein the fluid further comprising a thinning agent.

34. The component of claim 33 wherein the thinning agent is selected from the group consisting of thinning ester derived from soybean oil, thinning ester derived from palm oil, thinning ester derived from coconut oil, and alcohol.

35. The component of claim 33 wherein the thinning agent comprises from about 0% to about 30% by weight of the fluid.

36. The component of claim 27 wherein the oil is hydrogenated vegetable oil and wherein the hydrogenation of the oil is on the order of salad quality oil.

37. The component of claim 27 wherein the oil is hydrogenated vegetable oil and wherein the hydrogenated oil has an Iodine Value of approximately 100 to approximately 120.

38. A method of making an electrical component comprising:

creating an electrically-insulating fluid comprising a base oil selected from the group consisting of at least partially hydrogenated vegetable oil, vegetable oil higher in oleic acid content relative to a corresponding vegetable oil made from commodity grain, and combinations thereof, wherein the base oil is made from commodity corn oil which is partially hydrogenated.

39. The method of claim 38 wherein the fluid further comprises an antioxidant.

40. The method of claim 38 wherein the base oil comprises detectable to less than one hundred percent of the fluid.

41. The method of claim 40 wherein the electrical component is an electrical transformer.

42. The method of claim 41 wherein the electrical transformer is a electric utility transmission and distribution transformer.

43. The method of claim 38 wherein the electrical component is a fluid-filled electrical transmission cable.

44. The method of claim 38 wherein the base oil is replaced into the electrical component after draining it of petroleum-based oil.

45. The method of claim 39 wherein the antioxidant comprises from 0.02% to 1.0% by weight of the fluid.

46. The method of claim 38 wherein the base oil is winterized.

47. The method of claim 38 wherein the viscosity of the fluid is adjusted by blending a thinning substance into the fluid.

48. A method of making an electrical component comprising:

creating an electrically-insulating fluid comprising a base oil selected from the group consisting of at least partially hydrogenated vegetable oil, vegetable oil higher in oleic acid content relative to a corresponding vegetable oil made from commodity grain, and combinations thereof, wherein the base oil is made from genetically-engineered corn that is higher in oleic acid content relative to commodity corn.

49. The method of claim 48 wherein the fluid further comprises an antioxidant.

50. The method of claim 48 wherein the base oil comprises detectable to less than one hundred percent of the fluid.

51. The method of claim 48 wherein the electrical component is an electrical transformer.

52. The method of claim 51 wherein the electrical component is an electrical transformer.

**19**

**53.** The method of claim **48** wherein the electrical component is a fluid-filled electrical transmission cable.

**54.** The method of claim **48** wherein the base oil is replaced into the electrical component after draining it of petroleum-based oil.

**55.** The method of claim **49** wherein the antioxidant comprises from 0.02% to 1.0% by weight of the fluid.

**20**

**56.** The method of claim **48** wherein the base oil is winterized.

**57.** The method of claim **48** wherein the viscosity of the fluid is adjusted by blending a thinning substance into the fluid.

\* \* \* \* \*

UNITED STATES PATENT AND TRADEMARK OFFICE  
**CERTIFICATE OF CORRECTION**

PATENT NO. : 6,340,658 B1  
DATED : January 22, 2002  
INVENTOR(S) : Cannon et al.

Page 1 of 1

It is certified that error appears in the above-identified patent and that said Letters Patent is hereby corrected as shown below:

Column 16.

Line 60, please delete "butylhydro-" and insert -- butylhydro --.

Signed and Sealed this

Twenty-third Day of April, 2002

Attest:

Attesting Officer

JAMES E. ROGAN  
Director of the United States Patent and Trademark Office

